

## UNITED STATES PATENT OFFICE

1,932,835

## ALUMINUM ALLOYS

Ludwig J. Weber, New Kensington, Pa., assignor  
to Aluminum Company of America, Pittsburgh,  
Pa., a corporation of Pennsylvania

No Drawing. Application September 21, 1932  
Serial No. 634,151

2 Claims. (Cl. 75—1)

The invention relates to aluminum base alloys containing magnesium and silicon and to alloys of this type which have superior resistance to corrosive agents.

5 The alloys to which this invention has reference are of the general type which contain about 0.4 to 2.0 per cent by weight of magnesium, about 0.6 to 2.5 per cent by weight of silicon. The alloys contain at least about 93 per cent by 10 weight of aluminum and may, in addition, contain other alloying elements which may be added to the alloys to generally harden them or to produce therein other specific properties. Notable among such alloying elements are nickel, 15 manganese, etc. In the preferred form, these alloys are free from copper except as it may occur therein as an impurity, and it is to such alloys that this invention relates. Such alloys are of the type known to the aluminum arts as 20 strong alloys, i. e., their particular usefulness resides in their high strength and ductility, but these alloys have the further property of being comparatively resistant to corrosion, particularly in the heat-treated but unaged condition. 25 In normal condition and in the heat-treated and aged condition, these alloys are somewhat deficient in resistance to corrosion when compared with other aluminum alloys of lesser strengths. The alloys to which this invention has reference 30 are susceptible to thermal treatment, the most common of which is a heat-treatment at temperatures of above about 500° centigrade but below the temperature at which incipient fusion of the alloy takes place. This heat-treatment 35 may be followed by a rapid cooling and then by artificial aging which comprises heating the alloy to temperatures of about 100 to 200° centigrade to further develop the alloys' tensile properties. 40 With alloys of the above type I have experimented with the end in view of increasing their resistance to corrosion without materially detracting from the mechanical and other properties for which they are noted. I have finally determined that small amounts of the metal zirconium, when added to these alloys, directly 45 benefits their resistance to corrosive agents without materially affecting their mechanical properties or their workability. Nor does the addition of these small amounts of zirconium so 50 disturb the equilibria existing between the solid phases of the alloy as to decrease the known ability of the alloys to respond to commercial heat-treating methods. The amount of zirconium which achieves these results when added

to alloys of the type above described ranges from about 0.1 to about 1.0 per cent by weight of the total alloy. Zirconium is a metal which melts at relatively high temperatures and, therefore, I prefer to restrict the amount added whenever it is consistent with good results. About 0.2 to 0.3 per cent by weight of the total alloy is the preferred zirconium content. 60

Before explaining the beneficial effects produced in the above-mentioned alloys by the addition thereto of small amounts of zirconium, it will be necessary to briefly explain the nature of the corrosion which takes place in aluminum base alloys. All aluminum base alloys corrode to some extent when in contact with corrosive agents. This attack takes, *inter alia*, two general forms. It is usually either of the intergranular variety so named because the attack infiltrates into the alloy structure along grain boundaries, or it is of the "pitting" variety which does not proceed in any regular fashion and usually attacks only the metal surface. In aluminum base alloys of the type above described both varieties of attack occur in varying proportions and intensity depending upon the working and heat-treating history of the alloy. The intergranular type of corrosion is the most serious in that it tends to undermine the structure and, therefore, the strength and ductility of the alloy. 70 75 80 85

The addition of zirconium in the amounts above named to the alloys above described results in a general beneficial change in corrosion-resistance, but it also has the further and most beneficial effect of tending to reduce the amount of or the tendency to intergranular corrosion. This latter property of the zirconium is extremely beneficial and leads to measurable results. 90

For example, the following test results may be compared. In the table are shown the approximate compositions of four alloys. All alloys were in the form of rolled sheet when tested. Those alloys marked A had been heat-treated for about 15 minutes at about 515° centigrade and subsequently quenched in water. Those marked B 100 had a similar thermal treatment followed by cooling, but they were thereafter aged at 160° centigrade for about 18 hours. Each specimen was placed in an alternate immersion apparatus and alternately immersed and withdrawn from the corrosion solution in 3-minute cycles for a total period of 48 hours. They were then tested in comparison with other specimens of the same composition which had not been corroded. The corrosion solution was a standard one containing 105 110

about 5.3 per cent by weight of sodium chloride and 0.3 per cent by weight of hydrogen peroxide. In the table opposite the composition of each alloy is shown the tensile strength and elongation of the alloy before and after corrosion and the percentage change in these properties caused by the corrosion.

1. A metallic alloy consisting of about 0.4 to 2.0 per cent by weight of magnesium, about 0.6 to 2.5 per cent by weight of silicon, and about 0.1 to 1.0 per cent by weight of zirconium, the balance being substantially aluminum and the said alloy being free from copper except as an impurity.

80

| 10        | Composition |            |            |         | Tensile strength pounds per square inch |                 |                | Elongation—percent in 2 inches |                 |                | 85 |
|-----------|-------------|------------|------------|---------|-----------------------------------------|-----------------|----------------|--------------------------------|-----------------|----------------|----|
|           | Percent Mg  | Percent Si | Percent Zr | Balance | Before corrosion                        | After corrosion | Percent change | Before corrosion               | After corrosion | Percent change |    |
| 15 A----- | 0.6         | 1          |            | Al----- | 36,290                                  | 36,535          | +.7            | 28.5                           | 24.0            | -15.8          | 90 |
| B-----    | 0.6         | 1          |            | Al----- | 46,400                                  | 44,795          | -3.5           | 14.3                           | 5.50            | -61.5          |    |
| A-----    | 0.6         | 1          | 0.2        | Al----- | 35,060                                  | 35,015          | -0.1           | 26.3                           | 26.3            | 0              |    |
| B-----    | 0.6         | 1          | 0.2        | Al----- | 45,185                                  | 44,180          | -2.2           | 15.5                           | 14.5            | -6.5           |    |

20 A study of the properties shown in the table will demonstrate the effect of the presence of a small amount of zirconium. Those alloys containing no zirconium have deteriorated appreciably under the severe action of the corrosion test while those containing zirconium have deteriorated little if at all.

Having thus described my invention, I claim:

2. A metallic alloy consisting of about 0.4 to 2.0 per cent by weight of magnesium, about 0.6 to 2.5 per cent by weight of silicon, and about 0.2 to 0.3 per cent by weight of zirconium, the balance being substantially aluminum and the said alloy being free from copper except as an impurity.

95

100 LUDWIG J. WEBER.

30

105

35

110

40

115

45

120

50

125

55

130

60

135

65

140

70

145

75

150